

Patented June 5, 1923.

1,457,607

# UNITED STATES PATENT OFFICE.

CARL VON DER SCHMALZ, OF PHILADELPHIA, PENNSYLVANIA.

## WEIGHTING AND DYEING SILKS.

No Drawing.

Application filed August 10, 1922. Serial No. 581,027.

To all whom it may concern:

Be it known that I, CARL VON DER SCHMALZ, a citizen of the German Republic, residing at Philadelphia, in the county of Philadelphia and State of Pennsylvania, have invented certain new and useful Improvements in Weighting and Dyeing Silks, of which the following is a specification.

My invention relates to weighting and 10 dyeing silk, and the object thereof is to provide an improved silk and process of weighting and dyeing the same by means of non-injurious elements so as to produce weighted silk which is non-poisonous; which 15 obviates the use of a metallic salt or other chemicals which cause deterioration of the silk; which presents greater resistance of the dyed materials to the action of soap or a wash of soap and sodium carbonate; 20 greater strength of the fiber after dyeing, steaming, etc.; greater uniformity of the tints; which will permit weighting and dyeing of the silk in fabric, either alone or when combined with other vegetable or animal fibers; and which is sun-fast and light- 25 fast.

In carrying out the invention and treating, for example, one-hundred pounds (100 lbs.) of silk or silk combined with other 30 textiles, the process is as follows:

The first step consists in boiling off the silk in a 15% solution of olive soap with water.

The second step consists in dyeing the silk, 35 the dye stuff being at a boiling point of 212° F. and maintained at this temperature for one hour, after which 25% by weight of the silk treated, of Glauber's salt (sodium sulphate), is added. The material is left to 40 stand for one hour at the same temperature in this solution.

The third step consists in making the color fast with a 3% solution of formaldehyde, after washing or rinsing in cold water, to 45 which one pound (1 lb.) of chrome potash is added. The silk is allowed to stand in this solution for thirty minutes at 130° F. and particular care must be taken to avoid higher temperatures, unless it is desired to produce lighter shades, due to the 50 setting free of the formaldehyde at higher temperatures. The material is then rinsed or washed off again in cold water.

The fourth and important step consists in 55 combining with boiling hot water at the proportion of one hundred and twenty-five

pounds (125 lbs.) of sumac to 200 gallons of water or sixty-two and one half pounds (62½ lbs.) to 100 gallons of water, in which solution the silk is allowed to stand for 1½ hrs., after which it is removed and washed in clear cold water. The sumac may have combined therewith, 10% of tannic acid (C<sub>14</sub>H<sub>10</sub>O<sub>9</sub>), and is a non-poisonous vegetable matter of relatively high specific gravity in the form of a viscous syrup, either light or dark, according to the shade of the material to be treated. This treatment swells or expands the fibers and the solution penetrates and adheres to the same, to 70 produce a high grade weighted silk with a maximum of weight consistent with the treatment of the silk in fabric form as distinguished from the treatment of souple. 75

The last step in the process consists in 80 again soaking the silk in a 10% olive soap solution with water at 120° F., for thirty minutes, to give the necessary finish or lustre of silk, then washing the silk in luke warm water and then fresh or clear water at 100° F. to which is added 15% by weight of the 85 silk treated or fifteen pounds (15 lbs.) of 20% acetic acid to one-hundred pounds (100 lbs.) of the material treated and one-half pint of olive oil dissolved in one oz. of sodium carbonate to hold the oil in suspension and produce an emulsion to soften the 90 silk as well as produce the effect known as "scroup." The material thus treated is then stirred in fresh water and removed and dried. 95 In the case of hosiery, the material is passed through an extractor or in the case of piece goods, may be passed through a drier.

So far as I am aware, it is entirely new to employ sumac for the purposes stated 95 and particularly for weighting purposes in the treatment of silk. Light or dark shades of material may be treated and as an example, the silk may be treated alone either in knitted goods, such as hosiery, or in piece 100 goods, or the silk may be treated when combined with other vegetable or animal fibers. For instance, the silk may be combined with cotton and the process adapted for treating black silk hosiery with feet and tops of mercerized cotton without injuring the cotton. 105

In lieu of employing sumac, especially for light shades of silk, gall obtained as a decoction from gall nuts or gall apples may be used, in which respect the sumac and gall may be considered as equivalents. However, in employing gall nuts the last 110

step of the process consisting in treating the material with a solution of olive soap and water, is omitted and a half quantity of seven and a half pounds ( $7\frac{1}{2}$  lbs.) of acetic acid is used since light shades will be faded or ruined with a stronger solution. Silk treated according to this process especially as a result of the use of sumac or gall nuts, will have a fast color which is not affected by sunlight or water, thus rendering the silk capable of being washed without fading.

Having thus described my invention, what I claim as new and desire to secure by Letters Patent is:—

- 15 1. The herein described process of weighting silk fabrics consisting in subjecting the dyed fabrics to the action of a solution of a non-poisonous vegetable syrup containing tannic acid.
- 20 2. The herein described process of weighting silk fabrics consisting in subjecting the dyed fabrics to the action of a solution of a non-poisonous vegetable syrup containing tannic acid with tannic acid added.
- 25 3. The herein described process of weighting silk fabrics consisting in subjecting the dyed fabrics to the action of a solution of sumac with boiling water.

4. The herein described process of weighting silk fabrics consisting in subjecting the dyed fabrics to the action of a solution of sumac with boiling water with tannic acid added.

5. The herein described process of weighting silk fabrics consisting in subjecting the dyed fabrics to the action of a solution of sumac with boiling water in the ratio of from sixty to seventy pounds of commercial extract of sumac to one-hundred gallons of water.

40 6. The herein described process of weighting silk fabrics consisting in subjecting the dyed fabrics to the action of a solution of sumac in boiling water, soaking the fabrics in an olive soap solution, washing, treating with a solution of acetic acid with olive oil dissolved in sodium carbonate, rinsing in water and drying.

45 In testimony whereof I have signed my name to this specification in the presence of two subscribing witnesses.

CARL VON DER SCHMALZ.

Witnesses:

EDWARD J. HOLLAND,  
CHAS. E. POTTS.